

E. DANNER,  
APPARATUS FOR FORMING SHEET  
APPLICATION FILED APR. 11, 1917.

1,261,367.

Patented Apr. 2, 1918.  
7 SHEETS—SHEET 1.

Fig. 1.



INVENTOR.  
Edward Danner,  
By Owen, Owen & Crampton,  
His Atty.

1,261,367.

E. DANNER.  
APPARATUS FOR FORMING SHEET GLASS.  
APPLICATION FILED APR. 11, 1917.

Patented Apr. 2, 1918.  
7 SHEETS—SHEET 2.

Fig. 2.



INVENTOR.  
Edward Danner,  
By Burn, Owen & Crampton,  
His attys.

1,261,367.

E. DANNER,  
APPARATUS FOR FORMING SHEET GLASS,  
APPLICATION FILED APR. 11, 1917.

Patented Apr. 2, 1918.

7 SHEETS—SHEET 3

Fig. 3.



*INVENTOR.*

Edward Danner,  
By Burn, Cwin & Crampton,  
His attorney.

E. DANNER,  
APPARATUS FOR FORMING SHEET GLASS,  
APPLICATION FILED APR. 11, 1917.  
1,261,367.

Patented Apr. 2, 1918.

7 SHEETS—SHEET 4.

Fig. 4.



Fig. 5.

Fig. 6.



INVENTOR.  
Edward Danner,  
By Own, Brown & Crampton,  
His atlys.

E. DANNER.  
1,261,367.

APPARATUS FOR FORMING SHEET GLASS.  
APPLICATION FILED APR. 11, 1917.

Patented Apr. 2, 1918.  
1 SHEETS—SHEET 5.

Fig. 7.



Fig. 8.



1,261,367.

E. DANNER,  
APPARATUS FOR FORMING SHEET GLASS,  
APPLICATION FILED APR. 11, 1917.

Patented Apr. 2, 1918.  
1 SHEETS—SHEET 6.

Fig. 10.  
Fig. 11.



INVENTOR.  
Edward Danner,  
By Burn Burn & Crampton  
His atty.

E. DANNER,  
APPARATUS FOR FORMING SHEET GLASS.  
APPLICATION FILED APR. 11, 1917.  
1,261,367.

Patented Apr. 2, 1918.

7 SHEETS—SHEET 7.



Fig. 9.

INVENTOR.  
Edward Danner,  
By Burn, Burn & Crampton,  
His Atty.

# UNITED STATES PATENT OFFICE.

EDWARD DANNER, OF TOLEDO, OHIO.

## APPARATUS FOR FORMING SHEET-GLASS.

1,261,367.

Specification of Letters Patent. Patented Apr. 2, 1918.

Application filed April 11, 1917. Serial No. 161,210.

To all whom it may concern:

Be it known that I, EDWARD DANNER, a citizen of the United States, and a resident of Toledo, in the county of Lucas and State 5 of Ohio, have invented a certain new and useful Apparatus for Forming Sheet-Glass; and I do hereby declare the following to be a full, clear, and exact description of the invention, such as will enable others skilled 10 in the art to which it appertains to make and use the same, reference being had to the accompanying drawings, and to the characters of reference marked thereon, which form a part of this specification.

15 This invention relates to the glass working art, and particularly to the manufacture of sheet glass, and has for its object the provision of simple and efficient means for practising the process described in my 20 co-pending application Serial No. 95,070, filed May 3, 1916, for forming molten glass in continuous sheet form without the use of pressing or sizing rolls.

The invention is fully described in the 25 following specification, and while, in its broader aspect, it is capable of embodiment in numerous forms, a preferred and one modified form thereof are illustrated in the accompanying drawings, in which—

30 Figure 1 is a side elevation of the preferred form of apparatus for practising my invention with a part of the furnace broken away. Fig. 2 is a front end elevation thereof with a part broken away. Fig. 3 is a 35 section on the line 3—3 in Fig. 2 with glass being drawn in sheet form therefrom. Fig. 4 is a section on the line 4—4 in Fig. 3 with a part broken away. Fig. 5 is an enlarged side elevation of a portion of the 40 apparatus illustrating the slab adjusting means. Fig. 6 is a section on the line 6—6 in Fig. 5. Fig. 7 is an enlarged sectional detail of the slab shown in Fig. 3 provided with means at its free end for holding a 45 film of glass thereto. Fig. 8 is an enlarged fragmentary sectional view of the furnace similar to Fig. 3 and modified to illustrate a different form of slab onto which the molten glass flows. Fig. 9 is a front end 50 elevation of a different form of apparatus for practising the invention. Fig. 10 is a section thereof on the line 10—10 in Fig. 9. Fig. 11 is a section on the line 11—11 in Fig. 10, and Fig. 12 is a partial sectional 55 view of the apparatus with a different form

of drawing slab from that illustrated in Figs. 9 to 10, inclusive.

The practising of my invention, as set forth in said co-pending application, contemplates distributing molten glass evenly 60 on a slab which is disposed in a heated chamber, and drawing the glass in sheet form from the slab to stretch it to the desired thickness or size. For the practical and satisfactory drawing of sheet glass by my 65 process, it is important to maintain the slab, onto which the glass is first distributed and from which it is drawn in sheet form, highly heated so that the molten glass in flowing down the same is not permitted to too 70 quickly cool, and also to maintain the slab, or at least the greater portion thereof, in a high temperature so as to retard the external cooling of the glass surface as it flows down and is drawn from the slab. 75

In the apparatus illustrated in Figs. 1 to 6, 1 designates a furnace containing molten glass 2, which, in the present instance, flows from the furnace over a trough 3 into a practically closed chamber 4, that may be 80 heated by flames from a plurality of burners 5, if gas is employed as a fuel, such burners being arranged in suitable position within said chamber for an efficient heating of the same. The trough 3 terminates within the 85 chamber 4 and the flow of molten glass from its discharge end is regulated by a gate 6, which, for such purpose, is suitably mounted for vertical adjustment in the chamber 4 with respect to the trough. The gate 6, in 90 the present instance, has its upper end projecting without the furnace through the top of the chamber 4 and is carried by a plurality of stems or rods 7, which project upward from the upper end of the gate and 95 are threaded through the centers of adjusting wheels 8, which rest on the top of a frame work 9 at the top of the furnace. The wheels 8 on the separate rods 7 are in the form of sprockets and are connected by 100 a sprocket chain to cause a turning of the same in unison. A shaft 10 is vertically mounted in one side of the frame 9 and carries a hand-wheel 11 at its lower end and a sprocket-wheel 12 at its upper end. This 105 sprocket wheel is connected to a sprocket wheel 13, which is fixed to the adjacent sprocket-wheel 8 on one of the rods 7 to turn therewith. It is thus evident that a 110 turning of the hand-wheel 11 will effect a

simultaneous turning of the sprocket-wheels 8 on the several rods 7 and cause an adjusting of the gate 6.

- The molten glass is intended to flow in a 5 comparatively thin broad stream from the outer end of the trough 3 down onto the vertically registering surface of a slab 14, which is disposed in subjacent relation to the discharge end of the trough and rear- 10 wardly inclined to permit the glass to flow down the same by gravity in sheet form. The glass as it flows down the slab 14 is distributed evenly over the surface thereof and is partially cooled from the molten 15 state in which it flows from the trough 3 to give the glass sufficient consistency to enable it to be continuously drawn off in sheet form from the lower discharge end of the slab. Any suitable means, not shown, may 20 be provided without the furnace for imparting a continuous outward drawing movement to the glass sheet A, the speed of drawing being regulated to suit the thickness of the glass sheet required and the freeness 25 with which the glass flows down and from the outer end of the slab. It will be understood that the drawing of the glass from the slab causes the glass sheet to be stretched to the desired thickness.
- 30 The width of the glass sheet is partially regulated by side pieces 15 on the top of the slab 14 adjacent to its side edges, said side pieces being pivoted at their rear ends to the top of the slab, and their free ends 35 being movable inward or outward with respect to each other. Each side piece 15 has a rod 16 projecting outward therefrom transversely of the furnace through a sleeve 17 that is fixedly carried by the adjacent 40 end of the slab 14, a hand nut 18 being threaded on the rod 16 at the outer end of the sleeve 17 and prevented from longitudinal movements relative to the sleeve by a cage 19, which is fixed to the sleeve at its 45 outer end. It is evident that a turning of the nut 18 will effect an inward or outward adjustment of the side piece 15 with which it is connected.
- The slab 14 is disposed within a portion 50 4<sup>a</sup> of the chamber 4 at the lower forward part thereof and such portion of the chamber is heated by the flames from a plurality of gas burners 20 in its bottom. In order that the temperature within the chamber 4<sup>a</sup> 55 may be regulated to suit the conditions of drawing, which conditions vary for sheets of glass of different thickness, adjustable gates are provided above and below the outer end portion of the slab 14 and may be ad- 60 justed inward and outward to vary the size of the opening through which the slab projects, and also to expose a greater or less portion of the slab to the outside atmosphere or to an atmosphere which is cooler 65 than that of the chamber 4<sup>a</sup>. The upper

gate is designated 21 and is hingedly connected at 22 to the lower edge of a vertically movable plate 23 forming a portion of the front of the furnace chamber 4. The plate 23 is adjustably supported at its upper edges 70 by rods 24, which project up through sprocket wheels 25 that are threaded thereon and supported by the frame 9. The sprocket wheels 25 are connected by a chain 26 to cause a turning of the same in unison 75 and one of said sprocket wheels, which is of the double type, is connected by a chain 27 to a sprocket wheel 28 on a vertically disposed adjusting shaft 29. This shaft is journaled in vertical position in one side of 80 the frame 9 and carries a hand wheel 30 at its lower end.

Arms 31 project outwardly and downwardly from the lower edge portion of the plate 23 and carry a shaft 32 at their free 85 ends. This shaft is provided with a pinion 33 adjacent to each side arm, and each pinion is in mesh with a rack 34, which is pivotally connected at its inner end to the front side of the gate 21 whereby a longitudinal movement of the rack will effect a swinging adjustment of the gate. Each rack has a part thereof provided with a longitudinal slot 35 for receiving the shaft 32 and coöperates therewith to retain the 90 rack teeth in engagement with the associated pinion. The turning of the shaft 32 is controlled by the turning of the crank-shaft 36, which carries a worm 37 in mesh with a worm-wheel 38 on the shaft 32.

The gate which is disposed below the slab 14 is designated 39 and extends down at the rear of a shaft 40, that is mounted transversely in the base frame or truck 41 of the furnace. The gate 39 is provided on its 105 outer side adjacent to each end with a rack-bar 42, which extends transversely of the shaft 40 and meshes with a pinion 43 mounted thereon whereby a turning of said shaft will effect a vertical adjustment of the gate. 110 One end of the shaft 40 is provided with a worm-wheel 44 in mesh with a worm 45 on a shaft 46, which is journaled horizontally in one side of the frame 41 and carries a hand crank 47 at its forward end. The upper end of the gate 39 has a link 48 pivotally projecting rearward from each end thereof within the chamber 4<sup>a</sup> below the slab 14 and has its rear end provided with a slot 49 through which a transverse shaft 50 projects and carries a rack-bar 51 in mesh with a pinion 52 on said shaft. It is thus evident that a rocking adjustment of the gate 39 with respect to the shaft 40 as an axis may be effected by a turning of the shaft 50. The 120 shaft 50 extends at its ends without the furnace through horizontally elongated openings 53 (Figs. 1 and 5) in the side walls thereof and each end is journaled in a bearing block 54, which rests on a respective 130

bracket 55 for horizontal sliding movements transversely of the shaft, thus adapting the shaft 50 for transverse adjustment in a horizontal plane. The shaft 50 is provided at one end without the respective bearing 54 with a worm wheel 56 which meshes with a worm 57, the shaft of which carries a hand crank 58 and is journaled in bearing arms 59 projecting from the adjacent bearing 10 block 54.

Each block 54 has a rod 60 projecting rearward therefrom and threaded through a sprocket wheel 61 at the outer rear edge of the furnace chamber 4, said sprocket wheel 15 being connected to the sprocket wheel of the other rod 60 by a sprocket chain 62. Each sprocket wheel 61 is disposed within a cage 63 to prevent axial movements thereof. It is thus evident that a movement of the 20 sprocket chain 62 will effect a uniform adjustment of both bearing blocks 54.

The slab 14 is hung at its rear end on the shaft 50 for adjusting movements about the same as an axis, and is adjustably supported 25 at its forward end by a plurality of rods 64, which are mounted on the outer side of the gate 39 and guided for vertical movements thereby. The lower end portions of these rods thread through respective nuts 65 30 fixed to the gate 39, and the several rods have chain and sprocket connection 66 with each other, as best shown in Fig. 2, whereby the several rods are caused to have turning movements in unison. It is thus evident 35 that a turning of the rods 64 in the nuts 65 through which they are threaded will cause them to have uniform vertical movements and to raise or lower the outer or forward end of the slab 14 to vary the inclination 40 thereof and also to vary the size of the opening between the slab 14 and the gate 39, which tilting of the slab and regulating of such opening is desirable to meet the conditions and temperature of the glass being 45 worked.

It is evident from the foregoing that a rotary adjustment of the shaft 50 will effect an inward or outward movement of the upper end portion of the gate 39 due to the 50 rack and pinion connection of the links 48 of said gate with said shaft; that a transverse adjustment of the shaft 50 will move the slab 14 and gate 39 inward and outward in unison and that an adjustment of the 55 rods 64 will effect a raising or lowering of the outer end of the slab 14 and will increase or decrease the size of the opening between said slab and the upper edge of the gate 39.

In Fig. 7 the slab 14 is shown as being 60 provided adjacent to its outer or free edge with a passage 67, which extends from one end to the other of the slab adjacent to said edge and has a plurality of perforations 68 opening outward therefrom at the front 65 edge of the slab. The passage 67 has con-

nection with a suction creating means or source of vacuum so that a suction action is created through the perforations 68 and tends to draw and hold a film of glass to the front edge of the slab so that the glass sheet 70 will flow over said film as it is drawn from the slab. It is understood in the glass art that glass in a molten or liquid state will flow more readily over glass than over metal and for this reason vacuum is utilized to 75 hold a film of glass to the forward end of the slab so that the glass sheet passes over such film of glass as it leaves the slab. Another advantage of this feature is that the under surface of the glass does not have the 80 surface lines which are usually present when glass is drawn directly from a metal or clay surfaced slab.

In Fig. 8 the slab, which is designated 69, is disposed in substantially vertical position to permit the downward drawing of the glass sheet therefrom in a vertical plane. In this case the upper end portion of the surface of the slab on which the glass flows is rearwardly offset from the vertical portion 90 of such surface and stands in position for the molten glass to fall thereon as it flows from the trough 3, the glass then being distributed in sheet form over the surface of the slab and flowing downward therefrom. 95 The speed of drawing of the glass sheet from the lower end of the slab 69 is so regulated with respect to the speed of flow of glass down the face of the slab as to effect the desired sizing of the sheets. In other 100 words, the drawing means is intended to exert a pull on the glass sheet to assist the flow of the same from the slab and to stretch the sheet to the desired thickness or size. It is evident that with this form of 105 slab the surrounding atmosphere would need to be lower than that required if the slab was inclined, as otherwise the glass would flow too freely down the slab. The slab 69 is mounted in the same manner as described 110 for the slab 14 and the gates 21 and 39, and the rods 64 are adjusted to suit the position of the slab, as shown in Fig. 8. The glass sheet, if desired, may be drawn from the slab 69 down through the registering 115 portion of the truck frame 41 and an opening provided therefor in the floor or structure on which the frame 41 is mounted.

In the apparatus illustrated in Figs. 9, 10, 11 and 12, the slab is vertically disposed 120 and the molten glass is caused to flow down the same in a regulated stream which entirely surrounds or encompasses the slab. In this apparatus the trough 3, in which the molten glass flows from the furnace 1, 125 terminates at its outer end in a pot or tank 70 that is disposed within a heating chamber 71, which is heated, in the present instance, by flames from a plurality of gas burners 72. The pot 70 is elongated trans- 130

versely of the trough 3 to suit the width of the glass sheets to be drawn and is provided at its bottom with an elongated opening 73, which extends substantially the 5 length of the pot. A slab 74 of corresponding shape in cross-section to the opening 73 projects down through the opening and into a heating chamber 75, which is formed immediately below the bottom of the pot 70 by 10 a shell 76, which surrounds the slab 74 to near the lower end thereof.

The lower end of the heating chamber 75 is open to permit the flames, in the present instance, from a burner 77 to pass upward 15 therein from below the same and around the glass that is flowing down the slab 74, such flames finding an exit from the top portion of the chamber through openings 78 in the wall thereof. It is thus evident 20 that the flames from the burner 77, or the heat generated thereby, which rise around the glass as it flows downward from the pot 70 through the chamber 75, retards the cooling of the glass and permits it to be drawn 25 from the lower end of the slab 74 and sized as to thickness by the drawing stress which is applied to the glass without the slab.

The slab 74 is carried by hollow stems or tubes 79, which project up through the pot 30 and the top of the heating chamber 71, being provided above said top with sprocket wheels 80, which are threaded on said stems and rest at the lower ends of their hubs on a cross-beam 81 at the top of the furnace. 35 The sprocket wheels 80 are connected by a sprocket chain 82, and one sprocket wheel has chain and sprocket connection 83 with an adjusting shaft 84, whereby a turning of said shaft will effect a uniform turning of 40 the sprocket wheels 80 and a vertical adjusting of the slab 74. The head portion 85 of the slab is tapered or of wedge form whereby a raising or lowering thereof within the outlet opening 73 of the pot 45 effects a variation in the size of such opening to regulate the flow of molten glass from the pot.

If the lower end of the slab 74 is broad, or terminates with the side edges thereof 50 spaced, as shown, and air a little above atmospheric pressure is supplied to the interior of the drawing glass through the stems 79 and slab 74, the glass will be drawn in transversely elongated hollow 55 form, as shown at B, with opposing side walls thereof parallel and connected by short end portions. In such cases the short curved end portions of the drawing glass are severed from the side walls in any suitable manner, which forms no part of the 60 present invention and will therefore not be described, thus separating the drawn glass into two sheets of uniform thickness, size and quality.

65 If the lower end of the slab 74 is made

V-shape in cross-section, as shown at 74<sup>a</sup> (Fig. 12), and imperforate, the glass which flows down the slab at the opposite sides thereof will merge into a single sheet C as it passes from the slab, which sheet is drawn 70 to proper size after leaving the slab.

The chamber 76 is preferably vertically adjustable with respect to the slab 74, and for this purpose the wall 76 of the heating chamber is provided at opposite ends thereof with arms 86 through which extend rods 87 that project downward from the bottom of the furnace. A sprocket wheel is threaded on each of these rods in supporting relation to the arms 86 and are connected by 80 sprocket chains 88 to one member of a double sprocket wheel 89 threaded on a vertical rod 90 at one side of the rod 87. The other members of the sprocket wheels 89, 89 are connected by a sprocket chain 91. 85 It is thus evident that a movement of such chain will effect a simultaneous and uniform vertical adjustment of the sprocket wheels (not shown) which are carried by the rods 87. One advantage of mounting the shell 76 90 for vertical adjustment is to facilitate a replacing of the plate 92 which forms the opening 73 in the bottom of the pot 70.

It is evident in the use of each of the apparatus shown and described that the 95 molten glass is caused to flow in a molten state down a heated slab disposed in a heated chamber, the glass being distributed over the slab and flowing down and from the same in either single or multiple sheet form, the flowing of the glass from the slab being augmented by a drawing means which causes a stretching out and thinning or sizing of the sheet after leaving the slab. It will be understood that the thickness of the drawn sheet is dependent not only on the speed of drawing of the sheet from the slab, but also on the quantity of flow of molten glass from the trough 3 or pot 70, as the case may be, down the slab, and on the temperature maintained in the chamber within which the slab is disposed, it being evident that the lower the temperature within the slab containing chamber, the more quickly will the glass harden and set. As the glass 1 sheet is drawn from the slab and becomes hardened, it is severed into sections by any suitable means. Such severing, however, must take place at the outer side of the drawing means so that the drawn glass sheet 1 1 will be continuously maintained between the slab and drawing means.

It is evident that the sizing of the glass sheet or sheets is accomplished by the pull on the same and the temperature conditions of the chamber in which the slab is disposed and the quantity of flow of the molten glass down the slab, and that it is not necessary to pass the glass sheets between sizing rolls for such purpose. A further and very im-

portant feature of my manner of making continuous glass sheets is the increased speed with which the glass can be drawn, and the smoothness and uniformity in thickness of the product. It is evident that with the use of my apparatus it is not necessary to pass the glass between sizing rolls or for it to have contact with any roll or hard substance after leaving the slab and before the 10 glass is in a set condition, thereby preventing roughening of the glass surface which takes place by reason of such contact.

While I have herein shown and described several specific embodiments of my invention for illustrative purposes, it is to be understood that the invention is not limited to the mere details or relative arrangement of the parts, but that deviations from the illustrated forms or embodiments of the invention may be made without departing from the spirit of the claims.

Having thus described my invention, what I claim as new, and desire to secure by Letters Patent, is—

25 1. In an apparatus of the class described, a heated chamber having an outlet, and a slab having its discharge end lower than its receiving end disposed in said chamber in heat surrounded position and onto and down which molten glass may flow within the chamber and be drawn outward therefrom through said outlet in sheet form.

2. In an apparatus of the class described, a heated chamber, a slab having its discharge end lower than its receiving end disposed in heat surrounded position in said chamber, and means for permitting molten glass to flow onto the slab within the chamber and down the same, the glass being drawn in continuous sheet form from said slab.

3. In an apparatus of the class described, an inclined substantially flat slab surrounded by heat and having its discharge end lower than its receiving end, and means for permitting molten glass to flow onto and down said slab, the glass being drawn in continuous sheet form from the discharge end thereof.

50 4. In an apparatus of the class described, a chamber, a slab having its discharge end lower than its receiving end and disposed in said chamber and onto and down which molten glass may flow within the chamber and be drawn from the slab in sheet form, and means for creating a slab surrounding heat in said chamber with the heat diminishing toward the discharge end of the slab.

5. In an apparatus of the class described, 60 a heating chamber having an opening therein, a slab disposed within said chamber and projecting through said opening, said slab being surrounded with heat in said chamber, and means for directing molten glass onto said slab within the chamber, the glass

flowing down the slab and being drawn in continuous sheet form from the outer end thereof.

6. In an apparatus of the class described, a heated chamber having an opening therein, a slab within the chamber and onto which molten material may flow and be drawn lengthwise therefrom in continuous sheet form through said opening, and means for varying the size of the opening to regulate the temperature in the chamber.

7. In an apparatus of the class described, a heated chamber having an opening therein, an inclined slab within the chamber and onto which molten material may flow and be drawn lengthwise therefrom in continuous sheet form through said opening, said slab being surrounded with the chamber heat and having the surface thereof over which the material flows substantially flat in cross-section.

8. In an apparatus of the class described, a heated chamber having an opening therein, and a substantially flat slab adjustably mounted in said chamber and down which molten glass may flow and be drawn therefrom in continuous sheet form through said opening.

9. In an apparatus of the class described, a heated chamber having an opening therein, a slab mounted in said chamber for vertical swinging adjustment and down which molten glass may flow and be drawn lengthwise therefrom in continuous sheet form through said opening, and means for swingingly adjusting said slab.

10. In an apparatus of the class described, a heated chamber having an opening therein, a slab mounted in said chamber for vertical swinging and transverse axial adjustment and down which molten material may flow and be drawn lengthwise therefrom in sheet form through said opening.

11. In an apparatus of the class described, a heated chamber having an opening therein, a slab mounted in said chamber for vertical swinging and transverse axial adjustment and down which molten material may flow and be drawn lengthwise therefrom in continuous sheet form through said opening, and separate means for imparting different adjustments to said slab.

12. In an apparatus of the class described, a heated chamber having an opening therein, a slab disposed in heat surrounded position in said chamber and onto and down which molten material may flow and be drawn in continuous sheet form through said opening, and adjustable means on the surface of said slab for regulating the width of the glass sheet.

13. In an apparatus of the class described, a heated chamber having an opening therein, an inclined slab disposed in heat surrounded position in said chamber, means

- for permitting molten material to flow in a continuous stream onto and down said slab, the material passing from said slab in continuous sheet form through said opening, 5 and side pieces mounted on said slab and adjustable to regulate the width of the glass sheet flowing down the same.
14. In an apparatus of the class described, a heated chamber having a side thereof provided with an opening, a plurality of swinging gates adjustably restricting said opening, and a slab in heat surrounded position in said chamber onto and down which molten material may flow and be drawn through 10 said opening in continuous sheet form.
15. In an apparatus of the class described, a heated chamber having an opening in a side thereof, upper and lower gates mounted in said opening and forming a restricted 20 opening, said gates being swingingly adjustable to vary the size of said opening, and a slab disposed in heat surrounded position in said chamber in position for molten material to flow onto and down the same 25 and be drawn therefrom in continuous sheet form through said opening, the outer end of said slab projecting through said opening.
16. In an apparatus of the class described, 30 a heated chamber having an opening therein, a gate mounted for tilting adjustment and for adjustment transverse to its tilting axis to vary the size of said opening, and a slab in said chamber and onto which molten material may flow and be drawn lengthwise 35 therefrom in sheet form through said opening.
17. In an apparatus of the class described, a heated chamber having an opening there- 40 in, a gate adjustably mounted to restrict or enlarge said opening, means for imparting tilting adjustment to said gate, means for imparting adjustment to said gate trans- 45 verse to its tilting axis, and a slab disposed in said chamber and onto and down which molten material may flow and be drawn lengthwise therefrom in continuous sheet form through said opening.
18. In an apparatus of the class described, 50 a heated chamber having an opening therein, a reciprocally movable plate closing a portion of said opening, a gate hingedly carried by said plate and further restricting the size of said opening, separate means for vertically adjusting said plate and 55 swingingly adjusting said gate, and a slab disposed in said chamber and onto and down which molten material may flow and be drawn therefrom in sheet form through said restricted opening. 60
19. In an apparatus of the class described, a heated chamber, a slab tiltingly mounted in said chamber and onto and down which molten material may flow and be drawn therefrom in sheet form through said open- 65 ing, and means supporting the outer end of said slab and adjustable to vary the inclina- 70 tion of the slab.
20. In an apparatus of the class described, a heated chamber, a tiltingly mounted slab 70 disposed in inclined position in said chamber with its outer end projected through said opening, means for permitting molten material to flow onto and down said slab within said chamber and be drawn from its 75 outer end in continuous sheet form, a gate adjustably mounted below said slab to vary the size of said opening, and means carried by said gate for supporting the outer end of said slab and adjustable to vary the inclina- 80 tion of the slab.
21. In an apparatus of the class described, a heated chamber having an opening therein, a slab disposed in heat surrounding position in said chamber in register with said 85 opening, means for containing molten glass and permitting it to flow on said slab preparatory to passing down and being drawn from the slab in continuous sheet form, and means for regulating the flow of molten 90 glass onto said slab.
22. In an apparatus of the class described, a slab down which molten glass is permitted to flow and from which it is drawn, said slab having pneumatic suction means at its 95 outer end for drawing and holding a thin film of glass thereto.
23. In an apparatus of the class described, a slab down which molten glass is permitted to flow and from which it is drawn, said 100 slab having a plurality of openings at its outer end in communication with a source of vacuum to cause a drawing and holding of a thin film of glass to the slab end.
- In testimony whereof, I have hereunto 105 signed my name to this specification.

EDWARD DANNER.